

Patented Sept. 7, 1937

2,092,012

# UNITED STATES PATENT OFFICE

2,092,012

## ALUMINUM ALLOY

Joseph A. Nock, Jr., Tarentum, and George F. Sager, New Kensington, Pa., assignors to Aluminum Company of America, Pittsburgh, Pa., a corporation of Pennsylvania

No Drawing. Application November 25, 1936,  
Serial No. 112,760

4 Claims. (Cl. 75—142)

This invention relates to aluminum base alloys and it is particularly directed to improving the properties of certain alloys which contain the intermetallic compound,  $Mg_2Si$ , as the principal 5 hardening constituent.

Aluminum base alloys containing from about 0.5 to 3 per cent of the intermetallic compound  $Mg_2Si$  and lesser amounts of copper and chromium have been found to possess exceptionally 10 good cold working properties after thermal hardening treatment. In this respect they differ from many other aluminum base alloys which have received similar hardening treatment. Because 15 of these favorable characteristics the alloys have a wide field of application but their utility is limited under special conditions sometimes encountered in service where the corrosive attack is particularly severe, and where they are under high stress. It is particularly desirable that 20 under these conditions the alloys should have more than ordinary resistance to corrosive attack. Although these alloys are as resistant to 25 corrosion as many other aluminum base alloys, it is nevertheless very desirable in special applications that they should have a resistance to stress corrosion which is above the average for aluminum base alloys.

The term "stress corrosion" as herein employed refers to a type of corrosion in which the rate of 30 penetration is appreciably accelerated by the existence of a stress within the metal, especially where the stress is applied externally. This type of attack is generally distinguishable from that which ordinarily occurs on unstressed articles 35 both in rate and character. The two types of attack are not necessarily related since it has been found that a treatment or alloy addition may effectively inhibit ordinary corrosive attack and yet fail to afford protection against corrosion 40 under stress.

It is an object of our invention to improve the resistance to stress corrosion of aluminum-magnesium silicide-copper-chromium alloys of the composition herein set forth without impairing 45 their existing advantageous properties especially their working qualities. A further object is to accomplish this purpose in a simple direct manner without recourse to special treatment.

Our invention is predicated upon the discovery 50 that the addition of from 1 to 3 per cent zinc to an alloy composed of aluminum, 0.5 to 3 per cent of the intermetallic compound  $Mg_2Si$ , 0.1 to 0.75 per cent copper and 0.1 to 1 per cent chromium, materially improves the resistance to 55 stress corrosion. The use of zinc in the alloys within the aforesaid limits has no significant effect upon the cold working characteristics of the alloy nor does it impair the strength and hardness of the alloy in the solution heat treated and 60 precipitation-hardened or aged condition. As a

matter of fact the addition of zinc tends to increase the strength of the alloy as compared to that of an alloy of the same composition except for the omission of the zinc. The presence of zinc in the alloy offers an additional advantage 5 in that it combines with any magnesium in excess of the amount required to form the compound  $Mg_2Si$ , thus improving the resistance to ordinary corrosion. If an excess of uncombined magnesium is allowed to exist in the alloy, it has 10 been found that the resistance to ordinary corrosion will be impaired which is obviously undesirable.

We have found that the alloys containing the zinc are practically as workable as those without this element. They may be readily cold rolled, drawn or shaped either before or after the hardening thermal treatment. It is thus possible to make articles from the solution heat treated and aged alloys without danger of any warpage in 20 the finished product. The zinc does not appear to materially affect the workability of the thermally treated alloys.

In making the alloy, the proportion of magnesium and silicon should be so chosen as to insure 25 the formation of a maximum amount of the compound  $Mg_2Si$  with a minimum of either element in excess of that consumed in forming the compound. Under commercial operating conditions 30 it is not always possible to achieve this condition, generally because of slight variations in the silicon content of the base metal. Hence it is often desirable to add not more than about 0.1 per cent magnesium in excess of that which would ordinarily be required to combine with the estimated 35 amount of silicon. In this way, all of the silicon will be combined with the magnesium and thus insure a maximum amount of  $Mg_2Si$  which in turn will promote the development of the maximum strength throughout thermal treatment. 40 Any magnesium over and above that required to form  $Mg_2Si$  will unite with zinc to form a non-injurious compound. Magnesium and silicon have a greater affinity for each other than exists 45 between magnesium and zinc, and hence even though zinc is present in the alloy, yet the  $Mg_2Si$  compound will be formed first.

We have found that aluminum base alloys containing the compound  $Mg_2Si$ , and the elements copper, chromium and zinc in the proportions mentioned hereinabove, are especially well adapted to use in the manufacture of cold worked articles. In these alloys, the compound  $Mg_2Si$  should be the predominant alloying constituent aside from the aluminum, as well as being the 55 principal hardener. The copper and chromium only supplement the hardening effect of  $Mg_2Si$ . To obtain the optimum combination of properties in this type of alloy the following proportions of added alloying ingredients are preferred: 60

1.5 to 2.5 per cent  $Mg_2Si$ , 0.15 to 0.4 per cent copper, 0.25 to 0.75 per cent chromium, and 1.5 to 2.5 per cent zinc.

- 5 The heat treatment to which the alloy should be subjected to develop its maximum strength and hardness is of the conventional type, namely, heating at 500 to 530° C. until substantially complete solid solution is obtained whereupon the alloy is quenched or otherwise quickly cooled to room temperature. This treatment produces a considerable increase in strength, and for some purposes the alloys may be employed in this condition. However, the full strength and hardness can only be produced by reheating to 100 10 to 200° C. for a period of several hours. Since the alloys are primarily designed for use in the thermally treated form, they are rarely employed in any other condition. The improvement herein described is particularly effective in such thermal- 15 ly treated alloys.

The effectiveness of adding zinc to an aluminum base alloy containing the intermetallic compound  $Mg_2Si$  as the principal hardening constituent together with small amounts of copper and chromium, is illustrated by the following examples. Two alloys were made which had the nominal composition set forth in the table below. These alloys in the form of sheet 0.064 inch in thickness were given a solution heat treatment at 515° C., 25 quenched in water, and aged 18 hours at 160° C. The mechanical properties of these alloys in this condition were as follows:

| 35 | Percent composition |     |      |     | Lbs. per sq. inch |                | Percent elongation |
|----|---------------------|-----|------|-----|-------------------|----------------|--------------------|
|    | $Mg_2Si$            | Cu  | Cr   | Zn  | Tensile strength  | Yield strength |                    |
| 40 | 1.5                 | 0.2 | 0.25 | 1.5 | 40,700            | 33,800         | 12.3               |
|    | 1.5                 | 0.2 | 0.25 | 1.5 | 44,100            | 38,800         | 11.3               |

Uniform stress-cantilever specimens of the foregoing alloys were stressed at 75 per cent of their yield strength by fastening the base end

of the specimens in a fixture and applying a predetermined load at the other end which was unsupported and therefore free to move under the load. The specimens mounted in this manner were placed in an aqueous solution of 6 per cent NaCl, and an external electrical potential of 0.9 volt was applied, the specimens serving as anodes. The test was continued until the specimens failed to support the load. The specimens without zinc failed in an average time of 12 hours, whereas those containing zinc lasted for an average of 25 hours. The same observation has been made in other tests and thus confirms the fact that zinc has a very favorable effect in improving the stress corrosion resistance of the herein described 15 type of aluminum base alloy.

The term aluminum as used herein and in the appended claims includes metal containing the ordinary commercial impurities, although it also comprises a preferred grade of metal wherein the iron is held to a maximum content of 0.3 20 per cent.

We claim:

1. An aluminum base alloy consisting of aluminum, from 0.5 to 3 percent of the intermetallic compound  $Mg_2Si$ , 0.1 to 0.75 per cent of copper, 25 0.1 to 1 per cent of chromium, and 1 to 3 per cent of zinc.

2. An aluminum base alloy consisting of aluminum, from 1.5 to 2.5 per cent of the intermetallic compound  $Mg_2Si$ , 0.1 to 0.75 per cent of copper, 30 0.1 to 1 per cent of chromium, and 1 to 3 per cent of zinc.

3. An aluminum base alloy consisting of aluminum, from 1.5 to 2.5 per cent of the intermetallic compound  $Mg_2Si$ , 0.15 to 0.40 per cent of copper, 35 0.25 to 0.75 per cent of chromium, and 1.5 to 2.5 per cent of zinc.

4. An aluminum base alloy consisting of aluminum, 1.5 per cent of the intermetallic compound  $Mg_2Si$ , 0.2 per cent of copper, 0.25 per cent of 40 chromium, and 1.5 per cent of zinc.

JOSEPH A. NOCK, JR.  
GEORGE F. SAGER,